

1

3,487,088

PROCESS FOR PREPARING 1,3-DIMETHYLOL-4,5-DIHYDROXY-2-IMIDAZOLIDINONE

Kenneth Herald Remley, Warren Township, Somerset County, N.J., assignor to American Cyanamid Company, Stamford, Conn., a corporation of Maine  
No Drawing. Filed Apr. 14, 1967, Ser. No. 630,847  
Int. Cl. C07d 49/30

U.S. Cl. 260—309.7

1 Claim

ABSTRACT OF THE DISCLOSURE

A process for preparing stable aqueous solutions of 1,3-dimethylol-4,5-dihydroxy-2-imidazolidinone in which urea, glyoxal and formaldehyde are reacted under alkaline conditions of pH and at a temperature of from 30 to 130° C.

This invention relates to a process for preparing stable, aqueous solutions of 1,3-dimethylol-4,5-dihydroxy-2-imidazolidinone, sometimes referred to as dimethylol monourein or dimethylol dihydroxyethylenurea.

1,3-dimethylol-4,5-dihydroxy-2-imidazolidinone has the following structural formula:



The above imidazolidinone has become a valuable textile finishing agent particularly for use as a creaseproofing agent on cellulosic textile materials including blends of such materials with other fibers such as polyamides and polyesters. Although it may be employed as a conventional creaseproofing finish in the manner described in U.S. Patent No. 2,731,364, its present commercial importance is as a post-cure creaseproofing finish of the type employable in the process described in U.S. Patent No. 2,974,432.

At the present time there are three known processes for preparing 1,3-dimethylol-4,5-dihydroxy-2-imidazolidinone from urea, glyoxal and formaldehyde. All of the known processes are 2-step procedures.

In one, urea and glyoxal are reacted under alkaline conditions to produce 4,5-dihydroxy-2-imidazolidinone, which is then reacted with formaldehyde under neutral or alkaline conditions. (See U.S. Patents 2,731,472 and 2,764,573.)

In a second process, urea and formaldehyde are reacted under alkaline conditions to produce dimethylol urea which is then reacted with glyoxal under alkaline conditions to form the imidazolidinone. (See U.S. Patent No. 2,876,062.)

According to U.S. Patent No. 3,049,446, the product of the first process, that described in U.S. Patents 2,731,472 and 2,764,573, is dark brown and discolors cloth unless the intermediate monourein is purified before it is reacted with formaldehyde.

In the third process, urea and glyoxal are reacted at a pH of from 3.8-4.2, followed by reaction with formaldehyde at a pH of 7.0-7.5. (See British Patent No. 1,032,379.)

In all of the above processes the yield is generally low and the products contain large amounts of unreacted formaldehyde and glyoxal. In the case of the second process, that described in U.S. Patent No. 2,876,062, the product has been found to be unstable as evidenced by 70 discoloration on aging.

Accordingly, it is an object of the present invention

2

to provide a simplified, straight-forward process for preparing stable aqueous solutions of 1,3-dimethylol-4,5-dihydroxy-2-imidazolidinone that is characterized by good color, good stability and which is as effective as a creaseproofing agent for cellulosic textile materials as products prepared by the more costly two-step procedures of the prior art.

These and other objects and advantages of the present invention will become more apparent from the detailed description set forth hereinbelow.

According to the present invention, a process is provided for preparing a stable aqueous solution of 1,3-dimethylol-4,5-dihydroxy-2-imidazolidinone which comprises reacting relative amounts of 1 mole of urea with from between .8 and 1.3 moles of glyoxal and from 1.6 to 2.5 moles of formaldehyde in an aqueous medium at a pH maintained above 7 and at a temperature maintained between 30 and 100° C.

As described above, the present invention is concerned with a single step or "one pot" procedure for preparing what is substantially the equivalent in performance as a creaseproofing agent as similar products prepared by the more costly procedures of the prior art.

Preferably, the mole ratios employed are relatively amounts of 1 mole of urea with between .9 and 1.1 moles of glyoxal and between 1.8 and 2.2 moles of formaldehyde. Applicant has found that uniformly good results have been achieved by adhering to mole ratios within the preferred limits.

As indicated above, the aqueous reaction medium must be maintained above 7 and preferably between 7.5 and 9.5. The alkaline pH is obtained by adding sufficient alkali to provide the initial alkaline pH and by the continuous addition of suitable alkaline materials during the course of the reaction. Suitable alkalies include sodium hydroxide, potassium hydroxide, sodium carbonate and their equivalents.

As indicated above, the reaction mixture is heated at a temperature of between 30 and 100° C. and preferably between 60 and 70° C. It has been found convenient to permit the temperature of the reaction mixture to gradually rise until the desired reaction temperature is reached. The reaction temperature is maintained until it is essentially complete as evidenced by an unreacted aldehyde content of not over 2%, preferably not over 1.2%. The free formaldehyde content being determined by conventional analytical procedures.

When the reaction is finished the solution is normally cooled and sufficient acid added, preferably hydrochloric acid, to provide a pH of between 5.0 and 5.4.

If desired, sodium chloride or similar bleaching agents may be employed by addition to the aqueous solution to improve the color still further.

Textile finishes obtained by the procedure of this invention are stable, essentially colorless solutions. They are obtained economically and in excellent yield.

The products are applicable to cellulosic materials by known procedures and may be durably bound thereto by standard curing procedures. Cellulosic textile materials, illustratively cotton fabric, finished with the product of this invention have a high degree of wash-and-wear and other desirable properties, and are not discolored by the finish.

The product of this invention may be employed with other textile agents and auxiliaries such as softeners, brighteners, odorants and other creaseproofing agents.

In order to illustrate the present invention the following examples are given primarily by way of illustration. No specific details or enumerations contained therein should be construed as limitations on the present invention except insofar as they appear in the appended claims.

All parts and percentages are by weight unless otherwise specifically designated.

Example 1

To a suitable reaction vessel there is added 2,840 parts (41.6 moles) of 44% formalin and 3,000 parts (20.7 moles) of 40% aqueous glyoxal. Sufficient sodium hydroxide, about 55 parts of 24% aqueous caustic soda, is added to provide a pH of 8.0-8.5, followed by 1,250 parts (20.8 moles) of urea. The temperature of the reaction is allowed to rise to about 50° C. and 45 parts of 24% aqueous caustic soda is added. The temperature is then allowed to rise to 65-70° C. and is maintained at this level for two hours. During the two-hour period, additional amounts of sodium hydroxide are added as 24% aqueous sodium hydroxide in order to maintain the pH at 8-8.5. Thus 50 parts of 24% sodium hydroxide is added after 10 minutes, 25 parts after 30 minutes and 35 parts after one hour.

The reaction mixture is cooled to about 30° C. and 7 parts of sodium chlorite is added, followed by sufficient concentrated hydrochloric acid to provide a pH of 5.0-5.4. To the solution there is added 1,320 parts of water.

The product is an aqueous solution of 1,3-dimethylol-4,5-dihydroxy-2-imidazolidinone containing 45% solids and less than 1.0% of unreacted aldehyde. It is stable on storage and is suitable for application on textile materials without further processing.

Example 2

An aqueous pad bath is prepared containing 6.67% solids of the product in Example 1, 0.64% zinc nitrate, 3.0% of a nonionic softener, that is a 25% polyethylene emulsion containing polyethylene glycol monostearate and coconut oil monoethanolamine and 0.25% of a non-ionic surface active agent, that is the condensation product of nonylphenol with an average of 9.5 moles of ethylene oxide. Cotton broadcloth is impregnated with the pad bath by a standard padding procedure obtaining a 75% wet pickup. The fabric, containing 5.0% solids of the product of Example 1, is dried at 225° F. for one minute and then heated at 350° F. for 1.5 minutes.

Crease recovery angles of the treated and untreated fabrics are determined by AATCC Tentative Test Method 66-1959T.

The tensile strengths of the fabrics are measured by ASTM Standard Method D-39 using a Scott tensile strength tester.

The test results are shown in Table I.

TABLE I

| Fabric                                 | Untreated | Treated |
|----------------------------------------|-----------|---------|
| Crease recovery angle, W&F, degrees... | 188       | 58      |
| Tensile strength, W&F, lb.....         | 132       | 72      |

Example 3

An aqueous pad bath is prepared containing 10.2% of the product of Example 1, 0.98% of zinc nitrate, 3.0% of the nonionic softener and 0.25% of a nonionic surface active agent identified in Example 2,

Cotton/nylon twill (85%/15%) is impregnated with a pad bath by standard padding procedures obtaining a 60% wet-pickup. The fabric containing 6.1% solids of the product of Example 1 is dried at 225° F. for 1.5 minutes, steamed for 5 seconds, pressed on one side for 8 seconds and then on the other side for 8 seconds at 310° F. using 45 pounds/sq. in. pressure. The pressed swatches of cloth were heated at 320° C. for 10 minutes.

The crease recovery angles and tensile strengths of the treated and untreated fabrics are determined as indicated in Example 2.

The appearance ratings are relative, 5.0 being maximum, and are a measure of the smoothness of the fabric when viewed under an overhead light, after being washed five times.

The washes were carried out in a home-style washing machine using water at 140-145° F. and a detergent with a 12-minute wash cycle followed by tumble drying at 160° F. for 30 minutes.

The crease retention was determined by inspection of the fabrics after five wash and drying cycles.

The test results are shown in Table II.

TABLE II

| Fabric                                 | Untreated | Treated   |
|----------------------------------------|-----------|-----------|
| Crease recovery angle, W&F, degrees... | 154       | 278       |
| Tensile strength, F., lb.....          | 117       | 65        |
| Appearance rating.....                 | 1.8       | 4.8       |
| Crease retention.....                  | None      | Excellent |

I claim:

1. A process for preparing an aqueous solution of 1,3-dimethylol-4,5-dihydroxy-2-imidazolidinone comprising reacting in an aqueous medium, relative amounts of 1.0 mole of urea, between 0.9 and 1.1 moles of glyoxal and between 1.8 and 2.2 moles of formaldehyde at a pH maintained between 7.5 and 9.5 and at a temperature maintained between 60° and 70° C. until the reaction is essentially complete as evidenced by an unreacted formaldehyde content of not over 2%.

References Cited

UNITED STATES PATENTS

|           |         |                        |           |
|-----------|---------|------------------------|-----------|
| 2,731,472 | 1/1956  | Reibnitz -----         | 260-309.7 |
| 2,755,198 | 7/1956  | Stewart -----          | 260-309.7 |
| 2,764,573 | 9/1956  | Reibnitz et al. -----  | 260-309.7 |
| 2,777,857 | 1/1957  | König -----            | 260-309.7 |
| 2,876,062 | 3/1959  | Torke et al. -----     | 260-309.7 |
| 3,112,156 | 11/1963 | Vail et al. -----      | 260-309.7 |
| 3,209,010 | 9/1965  | Gagliardi et al. ----- | 260-309.7 |

HENRY R. JILES, Primary Examiner

NATALIE TROUSOF, Assistant Examiner

U.S. CL. X.R.

252-426; 260-77.5

55

60

UNITED STATES PATENT OFFICE  
CERTIFICATE OF CORRECTION

Patent No. 3,487,088 Dated January 22, 1970

Inventor(s) KENNETH HERALD REMLEY

It is certified that error appears in the above-identified patent and that said Letters Patent are hereby corrected as shown below:

Column 3, Table I, cancel "58" and "72" and substitute therefore --285-- and --76--.

SIGNED AND  
SEALED  
MAY 12 1970

(SEAL)

Attest:

Edward M. Fletcher, Jr.  
Attesting Officer

WILLIAM E. SCHUYLER, JR.  
Commissioner of Patents